

April 1, 1958

H. J. ROUND ET AL

2,829,047

MAGNETOSTRICTIVE ELEMENT

Filed April 2, 1954



HENRY J. ROUND AND Inventors  
KENNETH G. HINTON, DECEASED,  
BY FREDERICK H. HINTON, ADMINISTRATOR

By  
C. J. Deeler  
Attorney

# United States Patent Office

2,829,047

Patented Apr. 1, 1958

1

2,829,047

## MAGNETOSTRICTIVE ELEMENT

Henry Joseph Round, New Barnet, England, and Kenneth Gerald Hinton, deceased, late of Stratford-on-Avon, England, by Frederick Hubert Hinton, administrator, Stratford-on-Avon, England, assignors to The International Nickel Company Inc., New York, N. Y.

Application April 2, 1954, Serial No. 420,646

Claims priority, application Great Britain April 2, 1953

8 Claims. (Cl. 75—170)

Magnetostriuctive devices are used for the conversion of electrical to mechanical oscillations and vice versa, for example as transducers in echo-sounding apparatus. A measure of the efficiency of the magnetostriuctive device is given by its electromagnetic coupling coefficient (K). This coefficient may be determined experimentally and depends upon the material of the magnetostriuctive element.

The material commonly used for magnetostriuctive elements is commercially pure nickel, which combines a high electromagnetic coupling coefficient in magnetic fields of low and medium strengths with high resistance to corrosion.

An object of this invention is to improve the efficiency of magnetostriuctive devices.

The present invention is based on the discovery that the addition of small quantities of cobalt to the nickel improves the coupling coefficient at low and medium field strengths.

According to the invention, a magnetostriuctive element, for instance the vibrator of an echo-sounding device, is made of a binary alloy of nickel and cobalt containing from 2 to 6%, and preferably 4% cobalt. In making the alloys commercially pure nickel is normally used, and accordingly the usual impurities will also be present. Commercial nickel often contains very small quantities of cobalt, and on occasions the cobalt may be as high as 1.5%. The cobalt content of the alloys used according to the invention is higher than the highest amount of cobalt ever present as an impurity in commercial nickel.

The variation of the magnetic properties with the cobalt content is shown in the accompanying graphical drawing, in which the abscissae are the cobalt contents of nickel-cobalt alloys tested and the ordinates are the values of the coefficient K.

The curve shows the way in which the coefficient K was found to vary in one ring transducer. The coefficient was measured at a frequency of 33,000 cycles per second and at remanence, i. e. in the absence of an externally applied biasing magnetic field. It will be seen that pure nickel gave a value of K of 16%, and with 1% cobalt, which may be regarded as commercial nickel of rather high cobalt content, K was 20%. At 2% cobalt, however, K had risen to 24% and at 4% cobalt to 30%. As the cobalt content increased further the value of K began to fall again, being 23% at 6% cobalt. This graph is proof of the critical nature of the cobalt content, and of the advantage obtained by making the cobalt content from 2 to 6%, i. e. distinctly above that of any commercial nickel.

2

A substantially similar curve is obtained on measuring the maximum coefficient K in a biasing field.

We claim:

- 5 1. A transducer vibrator element exhibiting magnetostriuctive properties made of a binary alloy consisting of nickel and cobalt containing from 2 to 6% cobalt to provide high efficiency in the conversion of mechanical energy into electrical energy or vice versa.
- 10 2. A transducer vibrator element according to claim 1 in which the cobalt content is 4% to provide high efficiency in the conversion of mechanical energy into electrical energy or vice versa.
- 15 3. A transducer for converting mechanical energy into electrical energy or vice versa having a magnetostriuctive element consisting essentially of a binary alloy consisting of nickel and cobalt containing from about 2% to about 6% cobalt to provide high efficiency in the conversion of mechanical energy into electrical energy or vice versa.
- 20 4. A transducer for converting mechanical energy into electrical energy or vice versa having a magnetostriuctive element consisting essentially of a binary alloy consisting of nickel and cobalt containing about 4% cobalt to provide high efficiency in the conversion of mechanical energy into electrical energy or vice versa.
- 25 5. An echo-sounding device having a transducer for converting mechanical energy into electrical energy or vice versa having a magnetostriuctive element consisting essentially of a binary alloy consisting of nickel and cobalt containing from about 2% to about 6% cobalt to provide high efficiency in the conversion of mechanical energy into electrical energy or vice versa.
- 30 6. An echo-sounding device having a transducer for converting mechanical energy into electrical energy or vice versa having a magnetostriuctive element consisting essentially of a binary alloy consisting of nickel and cobalt containing about 4% cobalt to provide high efficiency in the conversion of mechanical energy into electrical energy or vice versa.
- 35 7. A transducer element exhibiting magnetostriuctive properties constructed of a binary alloy consisting of nickel and cobalt containing about 2% to about 6% cobalt to provide high efficiency in the conversion of mechanical energy into electrical energy or vice versa.
- 40 8. A transducer element exhibiting magnetostriuctive properties constructed of a binary alloy consisting of nickel and cobalt containing about 4% cobalt to provide high efficiency in the conversion of mechanical energy into electrical energy or vice versa.
- 45 9. A transducer element exhibiting magnetostriuctive properties constructed of a binary alloy consisting of nickel and cobalt containing about 4% cobalt to provide high efficiency in the conversion of mechanical energy into electrical energy or vice versa.

## 50 References Cited in the file of this patent

### UNITED STATES PATENTS

2,072,575 Acker ----- Mar. 2, 1937

### 55 FOREIGN PATENTS

3,448/26 Australia ----- May 13, 1927  
112,835 Australia ----- Mar. 31, 1941  
713,793 France ----- Aug. 24, 1931  
152,303 Switzerland ----- Apr. 1, 1932  
60 263,059 Great Britain ----- Dec. 18, 1926

### 60 OTHER REFERENCES

Ferromagnetism, by Bozorth, published by Van Nostrand, 1951, pages 672-674.